

## UNITED STATES PATENT OFFICE

2,622,278

## PREPARATION OF FILM CASTING SURFACES

Leopold Eckler, Summit, and William P. Moeller,  
Orange, N. J., assignors to Celanese Corporation  
of America, New York, N. Y., a corporation of  
Delaware

No Drawing. Application February 1, 1950,  
Serial No. 141,846

7 Claims. (Cl. 18—47.5)

1

This invention relates to film casting surfaces and relates more particularly to a novel process for preparing film casting surfaces that will produce films free from defects.

One of the processes heretofore employed for the production of films involves the flowing of dope containing a film-forming material, onto the surface of a casting member comprising a rotating, cylindrical casting drum having a diameter of from 10 to 18 feet, or more, and, after the dope has set, stripping the films from the drum. To obtain films free from defects, it has been the practice to provide the casting drum with a smooth, glossy casting surface by plating chromium, nickel or other corrosion-resistant metal thereon. The preliminary surface treatment of the casting drum to obtain a smooth and blemish-free deposit by plating and the plating operation itself are not only very cumbersome, but also extremely expensive and require a considerable period of time. Often the surface of the casting drum is damaged by scratches and other marks shortly after the final plating and must then be completely refinished.

To overcome the foregoing difficulties, it has been proposed to substitute for the plating on the casting drum a layer of gelatin or a cellulose ester coating. However, the application of these materials has not proved practical. In the case of gelatin, the joining of the ends of the layer is extremely difficult, as will be understood by those familiar with the art. As for the cellulose ester coating, the swelling, and particularly the uneven swelling, of the cellulose ester during the casting of films has proved a deterrent to its use.

In another prior process for the production of films, the dope containing the film-forming material is flowed onto the surface of a casting member comprising an endless belt disposed in a horizontal plane and trained over a number of pulleys. It has been proposed to provide this belt with a smooth, glossy casting surface by covering the same with a cellulose derivative coating, following which the surface of the cellulose derivative coating is chemically altered by treatment, for example, with a solution containing a de-esterifying agent. This process does not lend itself to the production of film casting surfaces on a casting drum. If a solution containing a de-esterifying agent is applied adjacent the top of a casting drum covered with a cellulose derivative coating, the solution will run down from the top of the drum in both directions and will produce streaks and other non-uniformities in the surface of the cellulose derivative coating.

On the other hand, a disassembling of the casting unit would be required to apply the solution to the bottom of casting drum.

Even in the case of a casting belt, longitudinal streaks are frequently produced during the treatment of a cellulose derivative coating with a solution containing a de-esterifying agent owing to the uneven application and mixing of the solution on various parts of the belt. A great deal of skill is also required in stopping and starting the application of the solution to avoid the production of very distinct marks on the film casting surface, which marks will be reproduced on the films cast thereon. Moreover, the treatment of the cellulose derivative coating with a solution containing a de-esterifying agent necessitates an extended washing to remove from the coating the excess of de-esterifying agent, during which washing there is a tendency to form flag marks on the coating which will be reproduced as defects in the films.

It is an important object of this invention to provide a process for preparing film casting surfaces which will be free from the foregoing and other disadvantages of the processes hitherto employed for this purpose and which will be especially simple and efficient in operation.

A further object of this invention is to provide a novel process for preparing film casting surfaces that will produce films free from defects.

Another object of this invention is the provision of a novel process for preparing on a casting drum film casting surfaces that will produce films free from defects.

Other objects of this invention will be apparent from the following detailed description and claims.

According to the present invention, a film-casting surface is prepared by covering the periphery of a casting drum, belt and the like with a cellulose derivative coating having a smooth, glossy surface, flowing a viscous dope containing a film-forming material and a reagent capable of chemically altering the cellulose derivative onto the cellulose derivative coating to form a film, and after the cellulose derivative has been chemically altered to the desired extent, stripping the reagent-containing film from the cellulose derivative coating to expose the film-casting surface which has been rendered solvent insoluble while retaining its smooth, glossy finish. This film casting surface may then be employed in conventional manner for the production of films. The process of the present invention may be carried out without modifying the equipment pres-

ently employed for the production of films by using the standard film-casting hopper for applying both the cellulose derivative coating and the reagent-containing dope to the casting member.

The reagent-containing dope may be applied on the cellulose derivative coating to form a film having one or a plurality of layers extending over the entire surface of the cellulose derivative coating. After the reagent has effected the desired change in the cellulose derivative, the reagent-containing film is stripped off, exposing the film-casting surface. Alternatively, the reagent-containing dope may be applied to the cellulose derivative coating as a single film which is stripped from the coating when it reaches the normal stripping point. In this event, the reagent-containing dope is applied to the cellulose derivative coating for a period long enough to obtain the desired change in the cellulose derivative.

As indicated, this invention may be employed for the preparation of a film-casting surface on a casting drum as well as on a casting belt. Owing to the viscosity and to the setting of the reagent-containing dope, the formation of streaks and other defects on the film-casting surface is eliminated. In addition, since it is no longer necessary to apply an excess of reagent to the cellulose derivative coating, the washing step hitherto employed for the removal of excess reagent may be dispensed with. The process of this invention requires much less time than the processes hitherto employed and, what is more important, leads to a greater and a more uniform depth of reaction. As a result of the greater depth of reaction, the film-casting surface is more durable since dust particles and fine scratches do not extend through the altered upper layers of the cellulose derivative coating and do not permit the access of solvent to the unmodified and solvent sensitive lower layers of the cellulose derivative coating. Blemishes in the surface of the coating, if they are not too deep, can, therefore, even be repaired without fear of reaching the solvent sensitive lower layer. By controlling the nature of the solvent or solvent mixture and quantity of reagent in the reagent-containing dope so that the solvent or solvent mixture evaporates and/or the reagent is exhausted before reaching too great a depth in the cellulose derivative coating, the reagent-containing film may be left in place to act as a protective layer until just prior to placing the casting unit in operation.

The cellulose derivative coatings employed in carrying out this invention may have a basis of a cellulose ester or mixed ester such as, for example, cellulose acetate, cellulose propionate, cellulose butyrate, cellulose-acetate propionate and cellulose acetate butyrate.

The cellulose derivative coatings may be chemically altered by de-esterification with any suitable reagents, e. g. alkaline materials such as potassium hydroxide, potassium or sodium alcohoholates, amines or quaternary ammonium hydroxide, for example. The viscous dope into which the reagents are incorporated may contain any suitable film-forming material that will not react with the reagents. For example, the dope may be prepared with ethyl cellulose, carboxy-methyl cellulose, methyl cellulose or an alkali soluble copolymer of styrene and maleic anhydride designated as Lustrex X-810. The dope may be prepared with any solvent or solvent mixture in which the reagent is soluble and in which the film-forming material may be dissolved or

dispersed, and which does not attack the cellulose derivative coating. The solvent or solvent mixture may have a swelling action on the cellulose derivative coating and aid the diffusion of the reagent into the coating and thereby help in the de-esterification of the cellulose derivative.

The dope may be applied to the cellulose derivative coating at room temperature or at an elevated temperature and may be made up with any desired concentration of reagent. The time of treatment will depend upon the character of the cellulose derivative coating, the temperature of the dope and the concentration of the reagent therein and may be varied to alter chemically the cellulose derivative coating to any desired depth.

The following examples are given to illustrate this invention further.

#### Example I

The surface of a casting drum is covered with a coating of methyl-cellulosolve-soluble cellulose acetate. Onto this coating, there are cast four superimposed layers of a dope containing 15% by weight of ethyl cellulose, and 0.6% by weight of potassium hydroxide in methanol. After drying, the ethyl cellulose film is stripped from the casting drum. The cellulose acetate coating is found to be de-esterified to a depth of 0.0045 inch.

#### Example II

The process of Example I is repeated, using a dope containing 15% by weight of ethyl cellulose and 0.4% by weight of sodium hydroxide in methanol. After stripping the ethyl cellulose film, the cellulose acetate coating is found to be de-esterified to a depth of 0.0003 inch.

#### Example III

The process of Example I is repeated, using a dope containing 15% by weight of Lustrex X-810 in water together with sufficient potassium hydroxide to dissolve the Lustrex X-810 and an excess of 1.5% by weight. After stripping the Lustrex X-810 film, the cellulose acetate casting is found to be de-esterified to a depth of 0.001 inch.

#### Example IV

The process of Example I is repeated, using a dope containing 5% by weight of carboxy methyl cellulose in water together with 0.5% by weight of potassium hydroxide. After stripping the carboxy methyl cellulose film, the cellulose acetate coating is found to be de-esterified to a depth of 0.001 inch.

It is to be understood that the foregoing detailed description is given merely by way of illustration and that many variations may be made therein without departing from the spirit of our invention.

Having described our invention, what we desire to secure by Letters Patent is:

1. In a process for the preparation of film-casting surfaces, the steps which comprise covering the surface of a casting member with a cellulose ester coating, and flowing a viscous dope containing a film-forming material and a reagent inert to said film-forming material and capable of de-esterifying the cellulose ester onto the surface of said cellulose ester to de-esterify the surface of said cellulose ester coating.

2. In a process for the preparation of film-casting surfaces for the reception of a solution of a film-forming composition in a volatile solvent therefor, the steps which comprise covering the surface of a casting member with a cellulose

ester coating, flowing a viscous dope containing a film-forming material and a reagent inert to said film-forming material and capable of de-esterifying the cellulose ester onto the surface of said cellulose ester coating to de-esterify the surface of said cellulose ester coating, and stripping the reagent-containing film from the cellulose ester coating to expose the film-casting surface.

3. In a process for the preparation of film-casting surfaces for the reception of a solution of a film-forming composition in a volatile solvent therefor, the steps which comprise covering the surface of a casting drum with a cellulose ester coating, flowing a viscous dope containing a film-forming material and a reagent inert to said film-forming material and capable of de-esterifying the cellulose ester onto the surface of said cellulose ester coating to de-esterify the surface of said cellulose ester coating, and stripping the reagent-containing film from the cellulose ester coating to expose the film-casting surface.

4. In a process for the preparation of film-casting surfaces, the steps which comprise covering the surface of a casting drum with a cellulose ester casting, flowing several superimposed layers of a viscous dope containing a film-forming material and an alkaline agent inert to said film-forming material and capable of de-esterifying the cellulose ester onto the entire surface of the cellulose ester coating to de-esterify the surface of said cellulose ester coating, and stripping the film containing the alkaline agent from the cellulose ester coating to expose the film-casting surface.

5. In a process for the preparation of film-casting surfaces, the steps which comprise covering the surface of a casting member with a cellulose acetate coating, and flowing a viscous dope containing a film-forming material and a reagent inert to said film-forming material and

capable of de-esterifying the cellulose acetate onto the surface of said cellulose acetate coating to de-esterify the surface of said cellulose acetate coating.

5 6. In a process for the preparation of film-casting surfaces, the steps which comprise covering the surface of a casting member with a cellulose acetate coating, flowing a viscous dope containing a film-forming material and an alkaline agent inert to said film-forming material and capable of de-esterifying the cellulose acetate onto the surface of the cellulose acetate coating to de-esterify the surface of said cellulose acetate coating, and stripping the film containing the alkaline agent from the cellulose acetate coating to expose the film-casting surface.

10 7. In a process for the preparation of film-casting surfaces, the steps which comprise covering the surface of a casting drum with a cellulose acetate coating, flowing several superimposed layers of a viscous dope containing a film-forming material and an alkaline agent inert to said film-forming material and capable of de-esterifying the cellulose acetate onto the entire surface of the cellulose acetate coating to de-esterify the surface of said cellulose acetate coating, and stripping the film containing the alkaline agent from the cellulose acetate coating to expose the film-casting surface.

15 LEOPOLD ECKLER.  
WILLIAM P. MOELLER.

## REFERENCES CITED

20 35 The following references are of record in the file of this patent:

## UNITED STATES PATENTS

| Number    | Name            | Date          |
|-----------|-----------------|---------------|
| 1,175,169 | Muller-Naegeli  | Mar. 14, 1916 |
| 1,988,550 | Gladhorn et al. | Jan. 22, 1935 |
| 2,353,717 | Francis et al.  | July 18, 1944 |